

Patented Jan. 27, 1925.

1,524,448

# UNITED STATES PATENT OFFICE.

JAMES A. MURPHY, OF LANSING, MICHIGAN.

## PLATING AND METHOD OF ACCOMPLISHING SAME.

No Drawing.

Application filed April 26, 1923. Serial No. 634,861.

To all whom it may concern:

Be it known that I, JAMES A. MURPHY, a citizen of the United States, residing at Lansing, in the county of Ingham and State of Michigan, have invented certain new and useful Improvements in Plating and Methods of Accomplishing Same, of which the following is a specification.

The object of my invention is to provide an improved plating and method of accomplishing same.

A further object of my invention is to provide a plating solution, which may be used in connection with the process of nickel plating which will eliminate a considerable part of the labor required for producing nickel plating, which will cheapen the cost thereof, which will decrease the time necessary for accomplishing the plating, which will eliminate one ordinary operation, and which will enable me to secure a coating of uniform thickness and texture.

In connection with the nickel plating process with which I have been familiar, and where it has been desired to secure a very high or the highest class of nickel plate finish on brass or ferrous articles, it has been customary to thoroughly clean the articles to be plated, then the articles if of a ferrous nature are copper plated, then polished, then nickel plated, and then the article is again buffed or polished, some polishing material being used in connection with the last buffing or polishing operation, which is designed to give the plated article what is termed "color". It is a further object of my invention to eliminate this last polishing or color operation in connection with nickel plating as the polishing operation or buffing tends to wear through the coating of plating at the corners or edges of the plated articles materially, thereby materially lessening the durability of the plate, as the greatest wear on such articles ordinarily comes on the corners or edges.

A further object of my invention is to provide a plating solution, which may be used in connection with nickel plating, and which will enable me to cut down the time ordinarily employed for plating. With these and other objects in view, my invention consists in the combination of the various ingredients of my compound or solution, and the method of using this solution for plating.

In the practice of my invention, I first

prepare the materials to be placed so that they are chemically clean. One way in which this may be accomplished consists of the following process: First, dipping the articles in a strong caustic lye solution; second, washing the articles by dipping them in a warm water bath of from 100 to 150 degrees Fahrenheit temperature; third, dipping the articles in an acid solution consisting of muriatic acid and water; fourth, washing the articles by dipping them in cool water, such for instance, as from 40 to 70 degrees Fahrenheit; fifth, immersing the articles for from one to three minutes in a cleaning device, using electrolysis and having an alkali solution therein, such for instance, as soda ash or tri-sodium solution therein; sixth, rinsing in cold water or cold water with a trace of muriatic acid therein; seventh, immersing in an alkali bath, using electrolysis if desired for a cleaner with an alkali solution with a trace of cyanide of potassium; eighth, dip in a cold solution of cyanide of potassium; ninth, rinse in cold water.

The tri-sodium solution above mentioned may be made of tri-sodium phosphate and water ( $Na_3PO_4$  plus 12  $H_2O$ ).

It will be understood that this method of cleaning is merely illustrative, and any suitable method of cleaning which will give a chemically clean surface may be used.

If the articles to be nickel plated are to be of a ferrous nature, it is desirable to first copper plate them, which may be done by immersing them in a copper solution in an electro plating tank, and plating for a period of time necessary to deposit a copper coating of the desired thickness.

Following the copper plating operations, if the articles are of a ferrous material or following the cleaning operation, if the articles are of a non-ferrous material, these articles are burnished or buffed on the surface to which it is desired to give a bright nickel finish. The extent of this burnishing or buffing process is dependent upon the smoothness of the final finish, which it is desired to produce, and may of course be continued until the metal has reached the desired smoothness.

Following the burnishing or buffing process described the articles are immersed in a nickel plating tank, containing the following solution: To one gallon of water add 8 ounces of nickel ammonium sulphate

$(\text{NiSO}_4 \cdot (\text{NH}_4)_2 \cdot \text{S. O}_4$ , plus  $6\text{H}_2\text{O}$ ), 4 ounces nickel sulphate ( $\text{NiSO}_4$ ) plus  $7\text{H}_2\text{O}$ ),  $\frac{1}{2}$  ounce salammoniac, 3 penny weights cadmium chloride,  $1\frac{1}{2}$  ounce glycerine.

- 5 The articles to be nickel plated are suspended in this solution which should be held in a temperature of from 70 to 80 degrees Fahrenheit, and should be maintained at a specific gravity of from 6 to  $8\frac{1}{2}$  Bé. The 10 specific gravity can be maintained for successive plating operations which tend to reduce same, by adding the metal parts of the solution thereto in the same proportions in which they are given in the above table. 15 A current voltage of from 1 to 5 volts may be maintained according to the amount and surface of the work which is being nickel plated, and the current should be maintained from 1 to 12 amperes per square 20 foot of surface being plated.

The articles to be plated are suspended in a plating solution mentioned from 15 minutes to  $2\frac{1}{2}$  hours depending upon the thickness of the coating desired and upon 25 the current voltage used, the amperage used and the strength of the solution. If a very heavy coating is desired, the time is proportionately lengthy and if a comparatively light coating is desired, the time is shortened. 30 With a large amount of material in the tank at the same time, the time has to be proportionately lengthened. Whatever the time may be that the article is allowed to remain in the solution, it will be bright 35 and have a very high lustre at the time, it is removed from the solution, and this lustre will be maintained without further polishing or buffing operations. As soon as the article is removed from the plating baths, 40 it is rinsed in cold water and dipped in a two to one solution of muriatic acid, then rinsed in cold water and then dipped in hot water mixed with whale oil or whale oil soap, which permits the finish to dry 45 without being spotted, and at the same time preserves the finish and imparts the color desired thereto.

Among the many advantages arising from my improved process, the main one is the 50 fact that the buffing or polishing operation, which follows the plating operation in the ordinary nickel plating process with which I am familiar, has been eliminated in connection with the use of my improved process, whereby the plating will be just as thick at the corners or edges of the plated articles as it is on the plain surface thereof, so that a plate of a given thick-

ness will wear a proportionately longer time. Of course further advantages result 60 in the decrease in cost due to the elimination of this final polishing or buffing operation. A second main advantage of the use of my solution, resides in the fact that I am enabled to cut down the time of the 65 immersion of the articles in the nickel plating solution to about half that necessary for other solutions with which I have been familiar.

These advantages in connection with the 70 saving of time, labor and cost, together with the improvement in the plating secured, do not in any way effect the desirability of the appearance of the plate. In fact, the color and the finish of the samples 75 which I have made up by my improved process are fully equal to any nickel plated articles which I have ever seen.

The composition of the solution matter is varied somewhat: For instance, the proportion of cadmium chloride may be varied from one to six pennyweights in the formula herein given. The proportions of the single and double sulphate nickel salts may be varied both in regard to each other, and 80 in regard to the balance of the formula by considerable quantities without departing 85 from my invention. Any suitable substances may be substituted for the boracic acid and the muriatic acid, which will accomplish 90 the same result, and the proportions thereof varied as much as 35% for instance, sulphuric acid may be substituted for muriatic acid and sulphate of aluminum for boracic acid.

Having thus described my invention, what I claim as new, and desire to secure by Letters-Patent, is:

1. A solution for a nickel plating tank comprising the following ingredients in the 100 proportions set forth, to one gallon of water, add from 5 to 12 ounces of nickel ammonium sulphate, 1 to 8 ounces nickel sulphate,  $\frac{1}{2}$  to 4 ounces boracic acid,  $\frac{1}{2}$  ounce sal-ammoniac 1 to 8 pennyweights cadmium 105 chloride,  $\frac{1}{8}$  to 2 ounces glycerine.

2. A solution for a nickel plating tank comprising the following ingredients in the 110 proportions set forth, to one gallon of water, add 8 ounces of nickel ammonium sulphate, 4 ounces nickel sulphate, 2 ounces boracic acid,  $\frac{1}{2}$  ounce sal-ammoniac, 3 pennyweights cadmium chloride,  $1\frac{1}{2}$  ounce glycerine.

In testimony whereof I affix my signature.  
JAMES A. MURPHY.